# EUROPEAN PATENT SPECIFICATION

(11) **EP 0 109 839 B1**
(45) Date of publication and mention of the grant of the patent: **06.09.1989**
(21) Application number: 83307051.9
(22) Date of filing: 18.11.1983
(51) Int. Cl.: H05B 7/085

(54) **Method of making graphite electrodes**
Herstellungsverfahren für Graphitelektroden
Procédé de fabrication d'électrodes en graphite

(30) Priority: 19.11.1982 US 443098
(43) Date of publication of application: 30.05.1984
(73) Proprietor: UNION CARBIDE CORPORATION, Danbury Connecticut 06817 (US)
(72) Inventor: Sara, Raymond Vincent, Parma Ohio 44130 (US)
(74) Representative: McCall, John Douglas

(56) References cited:
- EP-A- 0 063 710
- FR-A- 1 285 559
- FR-A- 2 133 802
- LU-A- 60 219

## Description

The invention relates to a unique process for manufacturing graphite electrodes for electric arc furnace applications and the unique electrodes resulting from the practice of the process.

Premium petroleum cokes are used extensively in the manufacture of electrodes for steelmaking with electric arc furnaces. The cost of such cokes is increasing very rapidly, however, and this could markedly affect the future growth of the use of electric arc furnaces and thus the market for electric arc electrodes. Less costly carbonaceous materials, such as anthracite coal, bituminous coal, lignites, so-called No. 2 coke, etc., have been tested in the production of electrodes intended for use in electric arc furnaces but the properties of the resulting electrodes are sufficiently inferior when compared to electrodes made from premium petroleum coke that they have been unacceptable for use in electric furnaces. Efforts to upgrade the properties of electrodes made from other than wholly petroleum coke as the carbonaceous source material to acceptable levels have been unsuccessful to date.

It has now been found possible to provide a method for manufacturing electrodes acceptable for use in electric arc furnaces in which the starting carbonaceous souce material is not premium grade petroleum coke.

According to the present invention there is provided a method of making an electric arc furnace graphite electrode which comprises calcining a carbonaceous material selected from anthracite coal, bituminous coal, lignites, and No. 2 coke, mixing the calcined carbonaceous material with the pitch, a lubricant, and a boron source selected from elemental boron, boron carbide, silicon tetraboride and iron boride, in an amount such that the boron content is from 0.1 to 5.0 perent by weight of the graphite electrode; extruding said mixture into an electrode form; and graphitizing said electrode form.

By "No. 2 coke" is meant ordinary or regular coke which is well known to be more or less amorphous and has a dark, spongy appearance, breaking into lumps of irregular shape.

The boron content of the graphite electrode is preferably substantially 3 per cent by weight of the electrode.

This invention resides in subjecting a carbonaceous source material, other than premium petroleum coke, and preferably anthracite coal, to the action of particular sources of boron, preferably boron carbide (B₄C), whereby the highly disordered structure of the carbonaceous material (preferably anthracite coal is transformed into one that is very graphitic in an otherwise conventional electrode manufacturing process.

By a preferred embodiment of the present invention there is provided a method of making an electrode suitable for use in an electric arc steel melting furnace which comprises hot mixing calcined anthracite coat particles, pitch, lubricants and boron carbide, such that boron is present in the amount of substantially 3 weight percent of the electrode, extruding said mix into an electrode form and heating said shaped electrode to graphitization temperatures.

In the practice of the present invention particles of the defined calcined non-petroleum coke carbonaceous material are mixed together with the conventional pitch binder and lubricant, and to this mixture is added the defined boron source. The boron source is one which does not release a gaseous byproduct when it is to be reacted with the carbonaceous material at the graphitization step in the manufacturing process and, as defined above, is selected from elemental boron, boron carbide (B₄C), silicon tetraboride (B₄Si) and iron boride (FeB).

15.24 cm (six-inch) diameter coarse-grain anthracite coal electrodes were formed by extrusion. The anthracite coal was calcined at 2200°C prior to crushing and sizing. The coal particles, pitch, lubricants, and B₄C additions to the mixes are indicated in Table I. The control mix had no boron, whereas the mix for the boronated stock was formulated to produce a finished product having approximately three weight percent boron.

The B₄C was Carborundum Company Technical Grade 325/F, containing seventy-two percent boron and a maximum particle size of 44 um. The B₄C and flour were blended in a ribbon blender for one hour prior to mixing with the other additions in a sigma-bladed heated mixer. A mix tempertaure of 158°C was achieved. The mix was then cooled to 110°C and extruded at 105°C. Extrusion pressures varied between 2689 and 3447 kPa (390 and 500 psi) for the control and between 2758 and 5576 kPa (100 and 800 psi) for the boronated mix. The higher extrusion pressure for the boron-containing mix indicates that insufficient binder was present, which should probably be detrimental to physical properties, especially strength. However, in spite of this, as shown in Table II, the boronated electrode had significantly higher strength than the control electrode. Eight billets measuring 15.24 cm (six inches) diameter by 45.72 cm (eighteen inches) long were formed from each mix.

The billets were packed with coke packing in saggers and baked at 2°C/hour to 500°C, at 10°C/hour to 900°C and held for approximately ten hours at the latter temperature.

Baked billets were then impregnated with Ashland 240 petroleum pitch. The procedure entailed preheating the billets in an autoclave to 225°C and evacuating the chamber thereafter one-half to one hour. The pitch was heated to 250°C and introduced and the system pressurized ton 698 kPa (100 psi). The impregnated billets were packed in coke packaging and rebaked at 10°C/hour to 750°C and held for twenty hours at the latter temperature.

The graphitization process consisted of heating inductively at a rate of 200°C/hour to 2000°C and at 400°C/hour to the final temperature of 3000°C. Hold time at 3000°C was one hour. During graphitization and cooling the stock is protected from oxidation by coke packing.

Properties obtained on the control and boronated anthracite coal specimens are shown in Table II. With the exception of the CTE, all properties were measured on 2.54 cm x 2.54 cm x 15.24 cm (1" x 1" x 6") specimens cut in the extrusion direction (WG) and normal to the extrusion direction (AG). The data are averages of nine AG and eleven WG specimens. The CTE data are essentially room temperature values and these measurements were made on 0.635 cm x 1.905 cm x 15.24 cm (0.25" x 0.75" x 6") bars.

The data in Table II indicate the boronated material has properties superior to those for the control in both billet directions. The WG CTE and WG resistivity for the boronated coal are significant improvements.

In addition to the foregoing advantages imparted by the employment of boronated anthracite coal over nonboronated anthracite coal, an electrode made with boronated anthracite coal exhibits exceptional resistance to oxidation. This is an important characteristic for electrodes which must perform satisfactorily in the exacting environment of an electric arc furnace.

It appears that, uniquely, boron causes the anthracite coal or other carbonaceous stock to retain its impurities; even after graphitization.

The principal impurities in anthracite coal are compounds of iron, silicon, aluminium, and titanium, and they equate to approximately ten percent ash. Most naturally occurring carbonaceous materials have as impurities similar kinds of elements in varying levels. The vaporization of these materials during graphitization results in lower density, poorer structure and properties. The presence of boron has been observed to prevent their vaporization. Impurities in the boronated carbonaceous stock provide excellent protection against oxidation. This phenomenon is clearly shown as explained below in the single Figure of the drawing.

The single Figure of the drawing is a graph illustrating the improvement in oxidation resistance of electrodes employing in their manufacture boronated anthracite coal as compared to electrodes employing non-boronated anthracite coal. The data illustrated in this graph was generated as follows: 2.54 cm (one-inch) cubes of the control and boronated anthracite coal stock were heated four hours in still air at temperatures between 800° and 1600°C. Material (carbon + ash) was weighed at the end of this time and the results are expressed as percent remaining in the Figure. The oxide coating developed in the coal specimens is a very small percentage (2-5 percent) of the remaining mass. Even at 1600°C, a substantial portion of the remaining material is carbon. At 1200°C, the control is almost completely oxidized, whereas approximately sixty percent carbon is retained in the boronated specimen. Accordingly, consumption will be much less for a boronated anthracite coal electrode exposed to electric arc furnace conditions than it would be for the unboronated counterpart.

The range of the amount of boron content to be added to the carbonaceous mix to be extruded into the finished electrode is between 0.1 and 5 percent by weight of the graphitized product, with about three percent being the preferred level of boron addition.

The properties of the boronated anthracite coal stock of the above example when compared to a graphite electrode made from premium petroleum coke are shown below in Table III.

As will be appreciated the properties of the electrodes of the invention compare very favourably with those that are available from conventional processing using premium petroleum coke.

Finally, it should also be appreciated that new, and lower cost electrodes suitable for use in electrical arc furnaces will also be achieved in those instances where the non-petroleum coke carbonaceous stock material which has been subjected to boronation replaces only a portion of the petroleum coke stock material rather than replacing it entirely.

## Claims

1. A method of making an electric arc furnace graphite electrode which comprises calcining a carbonaceous material selected from anthracite coal, bituminous coal, lignites, and No. 2 coke, mixing the calcined carbonaceous material with pitch, a lubricant, and a boron source selected from elemental boron, boron carbide, silicon tetraboride and iron boride, in an amount such that the boron content is from 0.1 ton 5.0 percent weight of the graphite electrode;. extruding said mixture into an electrode form; and graphitizing said electrode form.

2. A method according to claim 1, wherein the boron source is boron carbide.

3. A method according to claim 1 or 2, wherein the boron content of the graphite electrode is substantially 3 percent by weight of the electrode.

4. A method of making an electrode suitable for use in an electric arc steel melting furnace which comprises hot mixing calcined anthracite coal particles, pitch, lubricants and boron carbide, such that boron is present in the amount of substantially 3 weight percent of the electrode, extruding said mix into an electrode form and heating said shaped electrode to graphitization temperatures.

## Patentansprüche

1. Verfahren zur Herstellung einer elektrischen Lichtbogenofen-Graphit-Elektrode umfassend das Calcinieren eines kohlenstoffhaltigen Materials ausgewählt aus Anthrazitkohle, Fettkohle, Lignit (Braunkohlen) und Koks Nr. 2, Mischen des calcinierten kohlenstoffhaltigen Materials mit Pech, einem Gleitmittel und einer Quelle für Bor ausgewählt aus elementarem Bor, Borcarbid, Siliciumtetraborid und Eisenborid, in einer solchen Menge, daß der Borgehalt zwischen 0,1 und 5%, bezogen auf das Gewicht der Graphitelektrode, beträgt, Extrudieren dieser Mischung in eine Elektrodenform und Graphitglühen dieser Elektrodenform.

2. Verfahren nach Anspruch 1, bei dem die Quelle für Bor Borcarbid ist.

3. Verfahren nach Anspruch 1 oder 2, bei dem der Borgehalt der Graphitelektrode im wesentlichen 3 Gew.% der Elektrode beträgt.

4. Verfahren zur Herstellung einer Elektrode geeignet für die Verwendung in einem elektrischen Lichtbogenofen zum Schmelzen von Stahl, umfassend das heiße Mischen calcinierter Anthrazitkohlepartikel, Pech, Gleitmittel und Borcarbid, so daß Bor in einer Menge von im wesentlichen 3 Gew.% der Elektrode vorliegt, Extrudieren dieser Mischung in eine Elektrodenform und Erhitzen dieser geformten Elektrode auf Graphitisationstemperaturen.

## Revendications

1. Procédé de production d'une électrode de graphite destinée aux fours à arc électrique, qui consiste à calciner une matière carbonée choisie entre l'anthracite, le charbon bitumineux, des lignites et le coke N° 2, à mélanger la matière carbonée calcinée à un brai, un lubrifiant et une source de bore choisie entre le bore élémentaire, le carbure de bore, le tétraborure de silicium et le borure de fer, en une quantité choisie de manière que la teneur en bore représente 0,1 à 5,0% en poids de l'électrode de graphite, à extruder ledit mélange sous forme d'une électrode et à soumettre ladite électrode à une graphitisation.

2. Procédé suivant la revendication 1, dans lequel la source de bore est le carbure de bore.

3. Procédé suivant la revendication 1 ou 2, dans lequel la teneur en bore de l'électrode de graphite représente pratiquement 3% en poids de l'électrode.

4. Procédé de production d'une électrode convenant pour l'utilisation dans un four à arc électrique destiné à la fusion de l'acier, qui consiste à mélanger à chaud des particules d'anthracite calciné, un brai, des lubrifiants et du carbure de bore, de sorte que le bore soit présent en une quantité représentant pratiquement 3% en poids de l'électrode, à extruder ledit mélange sous forme d'une électrode et à chauffer ladite électrode façonnée aux températures de graphitisation.
